

## UNITED STATES PATENT OFFICE

CLIFFORD A. KAISER, OF CHICAGO, ILLINOIS

## METAL COILING

No Drawing.

Application filed September 24, 1931. Serial No. 564,981.

The present invention relates to metal coiling and has particular reference to the coiling of metal strips, sheets and the like in such a manner as to avoid defects such as coil breaks.

In the past it has been customary to process smelted metal to render the same suitable for manufacturing purposes by subjecting the metal in the form of bars, usually while hot, to processing in a hot mill. A hot mill unit consists essentially of one or two stands of rolls, a pair of furnace, one or more sheet furnaces and a squaring shear. The bars are heated in a pair furnace, passed back and forth through a stand of rolls, reheated in the sheet furnace when they are too cool for further working and are then finished by further passing back and forth through the rolls. The sheets formed in this manner vary in width from about 12 to 36 inches and in length from about 5 to 15 feet.

At the present time, this process is being superseded by the "continuous method". In this method, hot bars of a much greater size are started at one end of a series of from 2 to 10 or more mills and reduced in thickness progressively by each mill until they have been rolled out into long strips or strip sheets which may be one hundred feet or more in length. In order to facilitate handling, these sheets are customarily formed into coils.

In rolling mills using the continuous process for the manufacture of sheets, two methods are in general use for coiling the strip after it has been hot rolled or cold rolled.

In the "loose coiler" method the strip is passed through a set of three moving rolls so arranged as to cause the strip to attain a permanent deformation in the shape of a coil. Under present methods of manufacture, the inside diameter of the coil varies from approximately 20 to 30 inches, but, regardless of the inside diameter, there is a permanent deformation of the strip in the shape of a coil.

In the "tight coiler" method, the end of the strip is held between a set of jaws placed in a revolving drum. This drum pulls on the strip as it leaves the last stand of rolls, forming the strip into a coil approximately 30 inches in inside diameter. This method of coiling results in essentially the same kind of a coil as is produced by the "loose coiler".

Some rolling mills place the coilers as close as practical to the last stand of mills and if the strip has been rolled hot it is generally thought that coiling while still hot permits the sheet to acquire a certain amount of self annealing. Other mills do not coil the strip until the last portion of the strip has cleared the last hot mill stand, but no attempt is made to regulate the temperature of the metal during the coiling operation.

When such a coil is utilized for manufacturing purposes difficulty is encountered when the strip is being uncoiled. As the strip is uncoiled, it usually uncoils in a series of jerks, and at each jerk a bend occurs across the strip from one side to the other. This bend is what is known in the trade as a coil-break, and thus far, practically all attempts at eliminating coil-breaks have been directed toward preventing the jerking motion as the strip is being uncoiled.

A primary object of the present invention is to coil metal in such a manner that difficulties met with in utilizing the coiled strips are avoided.

An additional object is to produce a coil of metal which is not permanently deformed in the shape of a coil.

Still another object is to produce a metal coil, free from coil-breaks and other faults.

These and other objects will become apparent from the consideration of the following description.

My invention is based upon the discovery that, in the present method of coiling strips or sheets of metal, one surface of the strip or sheet is reduced and the other surface

is increased in length when the strip is coiled or uncoiled to such an extent that a series of failures occurs in the strip or sheet. If the strip is coiled hot, the failures occur when the strip is uncoiled, whereas, if coiled cold, the failures occur both while the strip is coiled and uncoiled. In accordance with my invention, these failures or coil-breaks are prevented by producing coils of a diameter sufficiently large that the surfaces of the strip will be neither stretched nor compressed an amount sufficient to cause a failure.

For stresses within the proportional limit, all elastic material, including metals, behaves according to the same law, namely, that the ratio of the unit-stress ( $S$ ) to the unit-strain or unit-deformation ( $e$ ) is a constant, or expressed mathematically,

$$20 \quad \frac{S}{e} = a \text{ constant,}$$

regardless of the kind of stress developed, whether tensile, compressive, or shearing, and regardless of the way the stress and deformation are produced, whether by axial, bending, or torsional loads. The numerical value of this constant ratio, however, is in general different for any one material when subjected to the different types of stress, and is also different for the different materials subjected to the same type of stress.

The numerical value of the constant ratio of the unit-stress in a material to the accompanying unit-strain within the proportional limit is called the modulus of elasticity of the material, and the symbol "E" is generally used to denote the modulus of elasticity.

For illustration, my invention will be described with particular reference to cold iron or steel, where the modulus of elasticity, or  $E$ , is approximately 29,000,000 pounds per square inch, both for tension and compression, and the proportional limit is about 29,000 pounds, depending on the composition and method of manufacture.

If a bar one square inch in cross section and 100 inches long is subjected to a stress, either tension or compression, it will be deformed. Applying a stress of 29,000 pounds, and solving the equation

$$\frac{S}{e} = E,$$

55 it is found that  $e$  equals 0.001 for a bar one inch long, or 0.1 for a bar 100 inches long.

Thus, if the stress be tension, the bar will be elongated to 100.1 inches, or, if compression, the bar will be shortened to 99.9 inches.

60 In either case when the stress is released the bar will go back to its original length.

If a stress of more than 29,000 pounds is applied to the bar, it will be distorted to more than 0.1, and will not regain its original length when the stress is relieved.

A strip .250 inch thick and 94.2480 inches long, the neutral axis of which will be a plane parallel to and midway between the two surfaces of the strip, when coiled, will make a cylinder having a neutral axis 30 inches in diameter. The inside surface of the coil, however, will be shorter than the neutral axis and the outside will be longer. The inside surface will be

75

$$\pi \times 29.7500 = 93.4626 \text{ inches,}$$

and the outside will be

$$\pi \times 30.2500 = 95.0334 \text{ inches.}$$

The difference from the neutral axis in either case amounts to .7854 inch. If a strip 94.2480 inches long be stressed up to its proportional limit, it will be deformed by only .09248 inch, or about 1/9th as much. Thus, where the strip is formed into a coil 30 inches in diameter, both the inside and outside surface of the metal is stressed beyond the proportional limit if the strip be coiled cold.

Consider, however, a strip .025 inch thick and also 94.2480 inches long. The circumference of the neutral axis is, as before, 94.2480 inches and the diameter is 30 inches. The inside diameter and circumference are, respectively, 29.9750 inches and 94.1695 inches, while the outside diameter and circumference are, respectively, 30.0250 inches and 94.3265 inches. The difference from the neutral axis in either case amounts to 0.07854 inch. From the equation

$$100 \quad \frac{S}{e} = E,$$

it is seen that  $S = 24,200$  lbs. per square inch. This is less than the proportional limit and the surface of the steel will not be permanently deformed. In accordance with my invention operation in this manner eliminates coil-breaks.

If a strip be coiled while hot (above 1,000° F. for steel) the aforementioned equation may or may not apply. When a strip is coiled hot, the physical and metallurgical characteristics are such that the individual grains of

which the metal is composed orient themselves in the new coiled formation while cooling and, when the coil is cool, any change in the form of the coil is met with the same amount of resistance as the cold, flat strip exerts when being coiled and, when stressed beyond the proportional limit, coil-breaks occur. Thus, a coil 30 inches in diameter and .250 inch thick will be stressed beyond the proportional limit when it is being straightened and the coil .025 inch thick will not.

In any case where a flat strip of metal is desired upon uncoiling, and coil-breaks are to be eliminated, I have found that it is necessary to coil the metal while cool as well as to form a coil having an inside diameter

100

105

110

115

120

125

130

135

140

145

150

155

160

165

170

175

180

185

190

195

200

205

210

215

greater than the diameter of coils produced heretofore.

I have further discovered that there is a definite relationship between the gauge of the metal to be coiled or uncoiled and the permissible diameter of the coil in order to prevent failure of the surface of either side of the sheet.

The increase in length of the outside of any coil, or the decrease in length of the inside from the length of the neutral axis which does not change is

$$\pi \times T, \text{ or } \pi \times (D_1 - D_2)$$

where  $D_1$  is the outside or inside diameter of the coil,  $D_2$  is the diameter of the neutral axis, and  $T$  is the thickness of the metal in inches. In order to keep within the proportional limit, the increase in length of the outside of the coil over that of the neutral axis must not be more than .001 inch per inch of length.

$$\frac{S}{e} = E \text{ or } e = \frac{29,000}{29,000,000} = .001 \text{ inch}$$

The increase in length of the outside =  $\pi \times T$ , and that must not be greater than  $.001 \times \pi \times D_2$  and solving for  $D_2$ , we find  $D_2 = 1,000 T$ , or in the case of steel, the diameter of the coil equals the thickness of the coil multiplied by 1,000.

As a general case, for any elastic material that is formed into a coil, in accordance with my invention the difference in length between the outside or inside surface of the coiled strip and the neutral axis should be equal to or less than the unit deformation multiplied by the length of the coil, or  $e \times \pi \times D_2$ . Since

$$e = \frac{S}{E}, \frac{S}{E} \times \pi \times D_2 = \pi \times T, \text{ or, } D_2 = \frac{E}{S} T,$$

where  $D_2$  is the diameter of the neutral axis of the coil,  $E$  is the modulus of elasticity of the material,  $S$  is the unit-stress in pounds per square inch, and  $T$  is the thickness of the strip or sheet in decimals of an inch.

For steel sheets or strips of various thickness, coils of not less than substantially the following diameters are required:

| Thickness of metal in inches | Diameter of circle in inches |
|------------------------------|------------------------------|
| .250                         | 250.00                       |
| .125                         | 125.00                       |
| .0625                        | 62.50                        |
| .050                         | 50.00                        |
| .0375                        | 37.50                        |
| .03125                       | 31.25                        |
| .025                         | 25.00                        |
| .01875                       | 18.75                        |
| .015625                      | 15.625                       |

The aforementioned figures apply to ordinary hot-rolled steel after it has been cooled and when it has a proportional limit of 29,000 lbs. per square inch. They will be altered somewhat on cold-rolled material having a

higher proportional limit, decreasing somewhat the diameter of coil necessary. For materials other than steel, the figures will be different, but the same principles apply and, in accordance with my invention, all elastic materials made into strips may be coiled in such a manner that failures such as coil-breaks are substantially eliminated.

I have found, therefore, that in order to prevent coil-breaks, it is necessary first to coil a strip to such a diameter that neither surface of the strip be stressed beyond the elastic limit, and that the strip be coiled at a temperature below that at which there is a rearrangement of the grains composing the metal due to the temperature. Consequently, the loose coiler method of forming metal strips into coils is unsuitable for use in accordance with my invention, since the loose coiler method causes a deformation of the metal beyond its elastic limit whereby the metal retains its coiled shape.

The utility of my invention is well demonstrated in the manufacture of sheets for materials or products such as metal furniture and the like where it is essential that the sheets have a certain degree of flatness. At the present time it is possible to obtain flat sheets from coiled strips only after subjecting the sheets to expensive further processing. In the old sheet mill process, after a sheet attained the required surface and degree of flatness, it was placed in a stretcher leveling machine and stretched beyond the elastic limit. The uniformity of the internal stresses within the sheet enabled the machine to stretch it uniformly over the entire sheet and, as a result, the sheet was stretched flat, or sufficiently so for the purpose for which it was intended.

After a sheet that has been made from a coiled strip has attained the required prerequisites as to surface finish and flatness, it too is stretcher-leveled. Few of the latter sheets pass inspection at the first stretcher-leveling and, therefore, they require additional processing. This additional processing usually consists of most or all of the following: annealing, pickling, roller-leveling, cold-rolling, and additional stretcher-leveling, thereby adding greatly to the cost of the finished product. Elimination of the aforementioned steps by operation in accordance with my invention means a material saving of time, labor and money.

Ordinarily, after a strip has been cold-rolled it is coiled either on a loose-coiler or tight-coiler as in hot-rolling. In this coiling, the strip is again stretched beyond the elastic limit on one side and compressed beyond the elastic limit on the other. As before, this introduces an internal stress within the strip and when the strip is cut into sheets and the sheets placed in a stretcher leveler to be stretched flat, the internal stress within the

sheet is not overcome by the external stretching force, thereby preventing the sheet from being made flat. In order to prevent this internal stress, it is necessary that the strip be coiled in such a manner and to such a diameter that, at no time will any portion of the strip be stressed beyond the elastic limit.

The various modifications of my invention which are not included in the foregoing illustrative and explanatory description are intended to be included in the appended claims.

I claim:

1. A method of treating metal which comprises heating the metal to a comparatively high temperature, rolling the heated metal into the form of a sheet, cooling the sheet to a temperature below that at which the grain structure is changed due to the temperature, and forming the cooled sheet into a coil having a diameter sufficiently large that the metal of the coil will not be stressed beyond its elastic limit when being coiled or uncoiled, said diameter being at least equal to the thickness of the sheet multiplied by 25 1,000.

2. A method of treating metal, which comprises forming the same into a sheet, and forming the sheet into a coil having a diameter sufficiently large that the metal of the coil will not be stressed beyond its elastic limit when being coiled or uncoiled, said diameter being at least as large as that derived from the formula

$$35 \quad D = \frac{E}{S} T,$$

where D is the inside diameter of the coil, E is the modulus of elasticity of the metal, S is a unit stress insufficient to reach or exceed the elastic limit of the metal, and T is the thickness of the metal sheet.

3. A method of treating metal, which comprises heating the metal to a relatively high temperature, rolling the heated metal into a sheet form, cooling the sheet to a temperature below that at which the grain structure of the metal changes due to the temperature, and forming the cooled sheet into a coil having a diameter at least as large as that derived 50 from the formula

$$D = \frac{E}{S} T,$$

where D is the inside diameter of the coil, E is the modulus of elasticity of the metal, S is a unit stress insufficient to reach or exceed the elastic limit of the metal and T is the thickness of the metal sheet, whereby said sheet does not acquire coil breaks when being coiled or uncoiled.

In testimony whereof I have hereunto subscribed my name.

CLIFFORD A. KAISER.